

## UNITED STATES PATENT OFFICE

EUGÈNE GAY, OF LYON, FRANCE

## PROCESS FOR OBTAINING PHOTOGRAPHIC IMAGES

No Drawing. Application filed October 14, 1926, Serial No. 141,671, and in France October 23, 1925.

In the specification filed upon a co-pending application Serial No. 141,670, dated 14th October, 1926, a process is described for obtaining photographic images based upon 5 the formation of azo dyes by reaction of diazo bodies sensitive to the action of light upon phenols or amines in the presence of alkali.

The invention consists in adding to the 10 diazo bodies forming the sensitive film or layer certain substances which produce phenols or naphthols by the action of alkalies, which permits sensitive films or layers to be obtained which can be developed by the 15 simple action of alkaline substances (vapours of ammonia or alkaline baths).

It has been established that the speed of 20 reaction of diazo bodies with phenols which is high in an alkaline medium is often far from negligible in a neutral medium and this constitutes an obstacle to the use of mixtures of diazo bodies with phenols for obtaining sensitive films or layers suitable for developing by the simple action of alkalies.

25 This disadvantage can be remedied up to a certain point by acidifying the mixture. Thus the speed of the reaction is diminished but this effect is secured to the detriment of the preservation of the substance of the support such as paper that is employed. In fact this leads with certain diazo bodies and certain phenols to the use of an inadmissible quantity of acid.

The difficulty referred to is obviated in 35 placing phenol or naphthol by one of its acetyl derivatives capable of regeneration under the action of the alkali employed during the development, which is introduced only at the moment of development.

40 The acetyl derivatives of phenols, di and tri-phenols, naphthols, dioxynaphthalines and amidonaphthols lend themselves particularly well to obtaining stable mixtures with diazo bodies in a neutral medium. The phenolic esters derived from formic acid, oxalic acid or benzene-sulphonic acid and generally 45 the aromatic bodies R. O. Ac. (in which R represents a benzene or naphthalene nucleus substituted or not substituted and Ac. denotes an acid radicle) may be employed. Certain

of these products being slightly soluble in water their sulpho or carboxyl derivatives may be used or even the alkaline salts of these derivatives. The diazo body and the acetyl derivative of phenol or naphthol are 55 mixed and the mixture used for the formation of the sensitive film or layer on the support, so that on exposure to light under a drawing or the like, the image, in azo colour, is produced by development of the exposed 60 film or layer by means of an alkali only.

Thus, for example, there is added to one litre of a bath of the diazohydroquinonedimethyl ether obtained according to the directions given in the specification filed upon the 65 said co-pending application, 30 gr. of 1-8-diacytdioxynaphthalene-3-6-disulphonic acid and one litre of water.

A sheet of paper or other convenient support impregnated in this bath, dried and exposed to light under a transparent design, until the parts not protected by the design are 70 decoloured, yields by development with the ammonia vapour a positive violet red image. The colour which constitutes the image is 75 identical with that obtained by coupling of the diazohydroquinonedimethyl ether and the chromotropic acid, that is to say, that it has the property of giving lakes with metallic salts, which permits of varying the shade 80 by trial either in toning them in baths of metallic salts after development or in introducing these salts in the sensitive bath.

I claim:

A process for obtaining a photographic 85 image of the kind described, consisting in impregnating a substance having a surface adapted for the reception of a photographic image in a bath of 1-8-diacytdioxynaphthalene-3-6-disulphonic acid and diazohydroquinonedimethyl ether, drying the said 90 substance and exposing the substance under a transparent design having substantially opaque parts and developing by an alkali to yield a positive violet red image, substantially as hereinbefore described.

EUGÈNE GAY.